

## UNITED STATES PATENT OFFICE

1,972,891

METHOD OF EXTRACTING DIPHENYL-  
AMINE

William T. Ingraham, Dover, N. J.

No Drawing. Application June 7, 1933,  
Serial No. 674,715

4 Claims. (Cl. 260—148)

(Granted under the act of March 3, 1883, as  
amended April 30, 1928; 370 O. G. 757)

The invention described herein may be manufactured and used by or for the Government for governmental purposes, without the payment to me of any royalty thereon.

5 This invention relates to a method of extracting diphenylamine and its derivatives from smokeless powder.

Smokeless powder that has deteriorated may be ground and reworked into new powder after 10 removing any free acid present. If the deteriorated powder is to be converted into a product such as nitrocellulose lacquer it is necessary to remove the diphenylamine and its nitro-derivatives as well as reduce the viscosity of the nitrocellulose. It is therefore proposed in the present 15 invention to provide a simple and economical method of removing diphenylamine and its derivatives from smokeless powder.

The method consists in grinding deteriorated 20 smokeless powder and treating it with a mixture of a solvent for diphenylamine which is a gelatinizing agent for nitrocellulose and an agent that prevents or retards gelatinization. An example of such a mixture consists of acetone and 25 water, the proportions to be employed depending upon the completeness of extraction desired, the length of time of soaking and the number of washes.

A preferred mixture consisting of 70% to 75% 30 acetone and 25% to 30% water, will give almost a complete extraction of the original diphenylamine present in the powder. Mixtures of equal parts of acetone and water have been successfully employed and slightly reduce the extent of removal of the diphenylamine.

The treatment is effected by allowing the comminuted powder to soak at room temperature and with or without agitation in one or more successive baths of the diluted acetone. The extent of extraction of the diphenylamine is influenced by the fineness of the powder, the number and length of the washes, and the proportion of the mixture. Examples are as follows:

In the first two examples given above the washing was conducted at 60° C., while in the others room temperature was used.

In no case does the solvent cause the smokeless powder to become swollen or adhesive and no difficulty is experienced in handling the powder during or after extraction.

Another advantage of the process is that it permits the reduction of the viscosity of the nitrocellulose in the powder without the use of a different solvent. This can be done by treating the powder, subsequent to the removal of the diphenylamine and its derivatives, with acetone containing a quantity of acetic acid.

I claim:

1. The method of treating smokeless powder containing diphenylamine which consists in comminuting the powder, and washing it at room temperature in one or more baths of a mixture composed of acetone 50% to 75% and water 75 50% to 25%.

2. The method of treating smokeless powder containing diphenylamine which consists in comminuting the powder, and washing it in one or more baths of a mixture composed of acetone 80 50% to 75% and water 50% to 25%.

3. The method of removing diphenylamine from comminuted smokeless powder which consists in submitting the powder to the action of a mixture of acetone 70% to 75% and water 25% 85 to 30%.

4. The method of removing diphenylamine from comminuted smokeless powder which consists in submitting the powder to the action of a mixture of acetone 50 to 75 parts and water 50 90 to 25 parts.

WILLIAM T. INGRAHAM.

| 45 | Fineness of powder | Mixture—acetone—water | Number of washes | First wash hours | Other wash hours | Total diphenylamine left in powder | Percent | 100 |
|----|--------------------|-----------------------|------------------|------------------|------------------|------------------------------------|---------|-----|
| 50 | 20                 | 50                    | 50               | 1                | 8                | -----                              | 0.30    | 105 |
|    | 20                 | 70                    | 30               | 1                | 8                | -----                              | 0.10    |     |
|    | 20                 | 70                    | 30               | 1                | 16               | -----                              | 0.23    |     |
|    | 20                 | 70                    | 30               | 7                | 16               | 2                                  | 0.02    |     |
|    | 20                 | 70                    | 30               | 4                | 16               | 2                                  | 0.04    |     |
|    | 30                 | 70                    | 30               | 3                | 16               | 2                                  | 0.01    |     |
| 65 | 48                 | 70                    | 30               | 3                | 16               | 2                                  | 0.02    | 110 |